

1

2,727,626

## FROTH FLOTATION

Lockwood W. Ferris, Salt Lake City, Utah, assignor to Compania Salitrera Anglo-Lautaro (Anglo-Lautaro Nitrate Corporation), New York, N. Y.

No Drawing. Application November 15, 1952,  
Serial No. 320,832

4 Claims. (Cl. 209—166)

This invention relates to the separation and separate recovery of water-soluble minerals or inorganic compounds by froth flotation. More particularly, the invention contemplates the provision of an improved process or method for treating a product containing or consisting essentially of solid sodium nitrate, solid potassium nitrate and solid magnesium sulphate heptahydrate to produce or obtain (1) a concentrate containing the potassium nitrate in predominant proportion or consisting essentially of potassium nitrate, (2) a concentrate containing the sodium nitrate in predominant proportion or consisting essentially of sodium nitrate and (3) a concentrate containing magnesium sulphate heptahydrate in predominant proportion or consisting essentially of magnesium sulphate heptahydrate.

Products containing mixtures of solid potassium nitrate, solid sodium nitrate and solid magnesium sulphate heptahydrate may be obtained in one or more stages of processes involving the recovery by solution and cooling or refrigeration of sodium nitrate from natural sodium nitrate-bearing deposits which contain potassium nitrate and magnesium sulphate associated with the sodium nitrate. The process of the present invention permits the separation and separate recovery of sodium nitrate, potassium nitrate and magnesium sulphate heptahydrate contained in precipitates obtained by cooling pregnant solutions thus providing for the recovery of three valuable products from a single product having little value as such. The precipitated products comprise or consist essentially of solid particles or crystals of sodium nitrate, solid particles or crystals of potassium nitrate and solid particles or crystals of magnesium sulphate heptahydrate.

The method or process of the present invention may be employed to effect separation of the precipitated sodium nitrate, potassium nitrate and magnesium heptahydrate and provide concentrate products of relatively pure sodium nitrate, relatively pure potassium nitrate and relatively pure magnesium sulphate heptahydrate. A complete separation operation to increase the purity of a concentrate with respect to its major component may be carried out in a multiple stage operation in which the separate concentrates obtained in any stage may be treated subsequently in accordance with a process of the invention.

In accordance with a method or process of the invention, (1) a solid product containing potassium nitrate, sodium nitrate and magnesium sulphate heptahydrate in large proportion or consisting essentially of potassium nitrate, sodium nitrate and magnesium sulphate heptahydrate is subjected in the form of an aqueous pulp saturated with respect to the components of the product and containing solid, finely divided particles of the product in suspension therein to a froth flotation operation in the presence of an organic cationic flotation reagent which functions as a mineral collecting agent to produce a potassium nitrate concentrate in the form of a froth and a concen-

trate of solid sodium nitrate and solid magnesium sulphate heptahydrate dispersed in finely divided form in the residual flotation pulp; (2) the potassium nitrate-bearing froth concentrate is separated from the residual flotation pulp; (3) the dispersed solid sodium nitrate and solid magnesium sulphate heptahydrate particles are separated from the liquid phase of the residual pulp, by filtration or otherwise, to obtain a product comprising a mixture of solid particles of sodium nitrate and solid particles of magnesium sulphate heptahydrate; (4) the resulting mixture of solid particles of sodium nitrate and magnesium sulphate heptahydrate in the form of a pulp free of the cationic reagent employed in producing the potassium nitrate concentrate but saturated with respect to the components of the original product comprising potassium nitrate, sodium nitrate and magnesium sulphate heptahydrate and containing the solid particles of the mixture suspended therein is subjected to a froth flotation operation in the presence of a half ester of a saturated monohydroxy alcohol such, for example, as sodium lauryl sulphate to produce a sodium nitrate concentrate in the form of a froth and a magnesium sulphate heptahydrate concentrate in the form of solid particles dispersed in the residual flotation pulp; (5) the sodium nitrate-bearing froth concentrate is separated from the residual flotation pulp; and (6) the solid magnesium sulphate heptahydrate particles are separated from the liquid phase of the residual flotation pulp to produce a solid magnesium sulphate heptahydrate concentrate.

The liquid phases of the residual flotation pulps may be utilized in carrying out additional froth flotation processes of the invention of the types of those of which they are products, or, they may be re-used in processes of the invention designed to improve the grades or qualities of the various concentrates involving re-treatment of the concentrates.

Any suitable organic cationic reagent may be employed as a mineral collecting agent in carrying out a method or process of the invention. Salts of alkylamines may be employed advantageously. In employing a salt of an alkylamine, I prefer to employ a salt in which the alkyl radical contains not less than eight and not more than eighteen carbon atoms. Alkylamine acetates may be employed with advantage. I have employed octadecylamine acetate with particular advantage.

Any suitable half ester of a saturated monohydroxy alcohol may be employed as a mineral collecting agent in a process of the invention for producing the sodium nitrate froth concentrate after separation of the potassium nitrate froth concentrate and after separation of residual solids from the liquid phase of the residual pulp and re-pulping of the residual solids.

For creating or assisting in creating froth at any stage of a process of the invention, I may employ any suitable frothing agent, but I prefer to employ an aliphatic alcohol having frothing properties. Such alcohols include the isomers of hexyl alcohol containing an isometric methyl group. Such isomers may be described as methyl amyl alcohols or as methyl pentanols. The alcohol designated or described as 3-methyl-1-pentanol or a mixture of methyl amyl alcohols containing a substantial proportion of that compound may be employed advantageously.

The product to be subjected to the froth flotation treatment may be ground to produce solid particles of any suitable sizes. Thus, for example, satisfactory results may be obtained by grinding to produce a finely divided product consisting of particles small enough to pass a 48-mesh screen. Grinding to produce a finely divided product consisting essentially of particles small enough

to pass a 100-mesh screen, however, results in economy in reagent costs and in a cleaner separation by froth flotation of the components of the original product.

The froth flotation method of the invention may be carried out with a pulp maintained at any suitable temperature. A temperature in the range of about 70° F. to 100° F. (or higher or lower if the atmospheric temperature at the point of location of the operation is higher or lower) may be employed advantageously.

A product of the following composition, typical of 10 precipitates produced in sodium nitrate recovery processes, was treated to demonstrate the effectiveness of the process of the invention:

| Component:                      | Percent by weight | 15 |
|---------------------------------|-------------------|----|
| Sodium nitrate                  | 36.0              |    |
| Potassium nitrate               | 39.1              |    |
| Magnesium sulphate heptahydrate | 23.4              |    |
| Moisture and impurities         | 1.5               |    |

In carrying out a typical test employing the method of the invention in treating a product of the above-indicated composition, five hundred (500) grams of the solid product were ground in a laboratory pebble mill containing brine in the form of an aqueous solution saturated with respect to the components of the product to form a pulp containing about sixty percent (60%) by weight of suspended solids consisting essentially of particles sufficiently small to pass a 100-mesh screen. The pulp produced in the pebble mill was transferred to a laboratory flotation cell and diluted therein with sufficient aqueous solution saturated with respect to the components of the product undergoing treatment to produce a pulp containing about twenty-five percent by weight of suspended solids. The diluted pulp was subjected to a froth flotation treatment in the flotation cell at room temperature in the presence of octadecylamine acetate ( $C_{18}H_{37}NH_2CH_3COOH$ ) in amount equivalent to eight-tenths (0.8) of a pound per ton of suspended solid particles and methyl amyl alcohol (3-methyl-1-pentanol) in amount equivalent to three-tenths (0.3) of a pound per ton of suspended solid particles. Agitation of the pulp with the added flotation reagents resulted in the production of a potassium nitrate froth concentrate substantially immediately. The froth produced was skimmed from the surface of the pulp in the flotation cell during a period of about five minutes. The residual pulp was removed from the flotation cell and filtered to separate the liquid and solid phases. The filter cake contained a large proportion of the sodium nitrate and magnesium sulphate heptahydrate of the original product and constituted a concentrate with respect to the sodium nitrate and magnesium sulphate heptahydrate. The filter cake solids were returned to the flotation cell and suspended in an aqueous solution saturated with respect to the components of the original product to form a flotation pulp containing about twenty percent (20%) by weight of suspended solids. The resulting pulp was subjected to a froth flotation treatment in the flotation cell in the presence of sodium lauryl sulphate in amount equivalent to eight-tenths (0.8) of a pound per ton of suspended solids and methyl amyl alcohol (3-methyl-1-pentanol) in amount equivalent to three-tenths (0.3) of a pound per ton of suspended solids. Agitation of the pulp with the added flotation reagents resulted in the production of a sodium nitrate-bearing froth concentrate substantially immediately. The froth produced was skimmed from the surface of the pulp during a period of about five minutes. The residual pulp was removed from the flotation cell and filtered to separate the liquid and solid phases. The filter cake contained a large proportion of the magnesium sulphate heptahydrate of the original product and constituted a concentrate of the magnesium sulphate heptahydrate with respect to magnesium sulphate heptahydrate (or a tailing product with respect to sodium nitrate and potassium nitrate).

The following tables show the compositions of the

three concentrates and the distribution of the components of the original product:

TABLE I

|                                                          | Percent<br>by Weight | Potassium<br>Nitrate,<br>Percent<br>by Weight | Sodium<br>Nitrate,<br>Percent<br>by Weight | Magnesium<br>Sulphate<br>Heptahy-<br>drate,<br>Percent<br>by Weight |
|----------------------------------------------------------|----------------------|-----------------------------------------------|--------------------------------------------|---------------------------------------------------------------------|
| Magnesium Sulphate<br>Heptahydrate Concent-<br>rate..... | 23.4                 | 1.60                                          | 3.9                                        | 94.2                                                                |
| Potassium Nitrate Con-<br>centrate.....                  | 40.0                 | 81.00                                         | 18.6                                       | 0.7                                                                 |
| Sodium Nitrate Concen-<br>trate.....                     | 36.6                 | 19.40                                         | 77.4                                       | 5.1                                                                 |

TABLE II  
*Distribution (percent by weight)*

|                                                     | Potassium<br>Nitrate | Sodium<br>Nitrate | Magnesium<br>Sulphate<br>Heptahy-<br>drate |
|-----------------------------------------------------|----------------------|-------------------|--------------------------------------------|
| Magnesium Sulphate Heptahydrate<br>Concentrate..... | 0.9                  | 2.4               | 94.2                                       |
| Potassium Nitrate Concentrate.....                  | 81.3                 | 20.3              | 0.7                                        |
| Sodium Nitrate Concentrate.....                     | 17.8                 | 77.3              | 5.1                                        |

I claim:

1. The method of separating potassium nitrate, sodium nitrate and magnesium sulphate heptahydrate contained in a solid product consisting essentially of potassium nitrate, sodium nitrate and magnesium sulphate heptahydrate which comprises subjecting the product in the form of an aqueous pulp saturated with respect to the components of the product and containing finely divided particles of the product suspended therein to a froth flotation operation in the presence of a salt of an alkylamine to produce a potassium nitrate concentrate in the form of a froth and a concentrate of solid sodium nitrate and solid magnesium sulphate heptahydrate dispersed in the flotation pulp, separating the froth from the flotation pulp, separating the dispersed solid sodium nitrate and solid magnesium sulphate heptahydrate from the liquid phase of the pulp to obtain a product comprising a mixture of solid particles of sodium nitrate and solid particles of magnesium sulphate heptahydrate, subjecting the resulting mixture of solid particles in the form of an aqueous pulp saturated with respect to the components of the original product comprising potassium nitrate, sodium nitrate and magnesium sulphate heptahydrate and containing the solid particles of the mixture suspended therein to a froth flotation operation in the presence of sodium lauryl sulphate to produce a sodium nitrate concentrate in the form of a froth and a magnesium sulphate heptahydrate concentrate dispersed in the flotation pulp, and separating the sodium nitrate froth concentrate from the flotation pulp.

2. The method of separating potassium nitrate, sodium nitrate and magnesium sulphate heptahydrate contained in a solid product consisting essentially of potassium nitrate, sodium nitrate and magnesium sulphate heptahydrate which comprises subjecting the product in the form of an aqueous pulp saturated with respect to the components of the product and containing finely divided particles of the product suspended therein to a froth flotation operation in the presence of a salt of an alkylamine to produce a potassium nitrate concentrate in the form of a froth and a concentrate of solid sodium nitrate and solid magnesium sulphate heptahydrate dispersed in the flotation pulp, separating the froth from the flotation pulp, separating the dispersed solid sodium nitrate and solid magnesium sulphate heptahydrate from the liquid phase of the pulp to obtain a product comprising a mixture of solid particles of sodium nitrate and solid particles of magnesium sulphate heptahydrate, subjecting the resulting mixture of

solid particles in the form of an aqueous pulp saturated with respect to the components of the original product comprising potassium nitrate, sodium nitrate and magnesium sulphate heptahydrate and containing the solid particles of the mixture suspended therein to a froth flotation operation in the presence of a half ester of a saturated monohydroxy alcohol containing not less than eight and not more than eighteen carbon atoms to produce a sodium nitrate concentrate in the form of a froth and a magnesium sulphate heptahydrate concentrate dispersed in the flotation pulp, and separating the sodium nitrate froth concentrate from the flotation pulp.

3. The method as defined in claim 2 wherein the salt of an alkylamine is an acetate of an alkylamine in which the alkyl radical contains eight to eighteen carbon atoms.

4. The method as defined in claim 2 wherein the salt of an alkylamine is octadecylamine acetate.

5 10 15 2,120,217 2,297,664 2,222,330 Harris Tartaron Weinig June 7, 1938 Sept. 29, 1942 Nov. 19, 1940

## 6 References Cited in the file of this patent

### UNITED STATES PATENTS

2,120,217 Harris June 7, 1938  
2,297,664 Tartaron Sept. 29, 1942  
2,222,330 Weinig Nov. 19, 1940

### OTHER REFERENCES

Taggart: Handbook of Mineral Dressing, John Wiley & Sons, 1945, pp. 12-02; 12-14 to 12-18, 12-40 to 12-43; 12-112; 12-116; 12-124, 12-125.

Chemiker Zeitung, Mar. 1, 1939, No. 17, pp. 148-149, Translation in Division 55. Soluble Salts, 9 pages.

Russian Patent 47,678, extract translation from "Report of the Committee on Inventions" (Vestnik Komitets po izolretatel' stvu), No. 7, July 31, 1936, in Division 25, 209-166, Soluble Salts, 1 page.